

## UNITED STATES PATENT OFFICE.

JOSEPH SEYER, OF HAWTHORNE, NEW JERSEY, ASSIGNOR TO STANDARD SILK DYE-  
ING CO., OF PATERSON, NEW JERSEY, A CORPORATION OF NEW JERSEY.

## WASHABLE BLACK SILK PIECE GOODS AND PROCESS OF DYEING THEM.

No Drawing. Original application filed December 1, 1922, Serial No. 604,390. Divided and this application filed February 24, 1923. Serial No. 621,075.

To all whom it may concern:

Be it known that I, JOSEPH SEYER, a citizen of the United States, a resident of Hawthorne, in the county of Passaic and State 5 of New Jersey, have invented certain new and useful Washable Black Silk Piece Goods and Processes of Dyeing Them, of which the following is a specification.

This invention relates to a new article 10 of manufacture or product consisting of washable black silk, and more particularly to a washable black fabric which has been dyed in the form of piece goods and it relates also to the process of producing and 15 dyeing such silks and silk fabrics.

This application is a division of my original application Serial Number 604,390, filed December 1, 1922, Patent Reissue No. 16,016, and it particularly covers process 20 #5 as described in my original application.

For producing a black on silk I proceed as follows: Silk piece goods are dyed in a bath composed of five hundred gallons water, 30% by weight of fustic extract, 10% 25 by weight of hematine extract (oxidized logwood). The goods are worked in the liquor at the boiling temperature for twenty minutes, and then to the same liquor are added 25% by weight of black iron, 4% by 30 weight of blue stone, and 20% by weight acetic acid (to dissolve precipitate in the bath). The goods are worked at the boiling temperature for one hour, and are then washed well. The goods are now treated 35 in another bath composed of five hundred gallons boiling water, 30% hematine extract, and fifty pounds soap, and they are worked therein for one hour and then washed. The next step consists in treating the goods in 40 a bath of five hundred gallons water at 160° F., containing tannic acid in the proportion of six pounds tannic acid per two hundred fifty gallons of dye liquor. This is followed by the tartar emetic treatment 45 as in process #3, namely, four and one-half pounds of tartar emetic per two hundred fifty gallons of dye liquor. The final dyed goods are given two cleansing soap baths at a boiling temperature, and then washed 50 well and acidulated.

There is thus produced a washable black which will not impart a black or dark color to a washing soap liquid below 160° F. or

thereabouts. A characteristic of my black silk piece goods is that they will not "bleed" 55 in cold water, that is, impart black thereto, nor will they readily show the marks and effects of perspiration. They may be washed together with silk, cotton, artificial silk, wool, etc. without staining them, the 60 temperature being about 110° F. They also have excellent fastness to light and ironing.

While my silk piece goods have been described as being of unmixed silk, it is also possible to make mixed silk goods, such as silk and cotton, by the above described process. It is to be understood that where exact temperatures and working conditions are given, it is merely for the purpose of 70 presenting a preferred embodiment and giving accurate directions, as variations may be made according to circumstances.

As many apparently widely different embodiments of my invention may be made without departing from the spirit thereof, 75 I do not intend to limit myself to any particular embodiment except as indicated in the following patent claims.

I claim:

1. The process of producing washable 80 black silk piece goods comprising dyeing them black in a hot liquor, and then fixing the dye with tannic acid and tartar emetic.

2. The process of producing washable 85 black silk piece goods comprising dyeing them black in a hot liquor, and then fixing the dye with tannic acid and tartar emetic, and thereafter cleansing the goods in a hot soap liquor.

3. The process of producing washable 90 black silk which comprises dyeing it black with a logwood extract and an iron salt in a continuously boiling liquor, and fixing the dye on the silk in a hot liquor containing tannic acid.

4. The process of producing washable 95 black silk which comprises dyeing it black in a continuously boiling liquor, and fixing the dye on the silk and treating the silk in a hot soap liquor.

5. The process of producing washable 100 black silk piece goods which comprises dyeing it black with a logwood extract and an iron salt in a continuously boiling liquor, and fixing the dye on the silk in a hot liquor.

6. The process of producing washable black silk piece goods which comprises dyeing it black with a logwood extract and an iron salt in a continuously boiling liquor, 5 and fixing the dye on the silk in a hot liquor containing tannic acid.
7. The process of producing washable black silk piece goods which comprises dyeing it black in a continuously boiling liquor, 10 and fixing the dye on the silk and treating the silk in a hot soap liquor.
8. The process of producing washable black silk piece goods which comprises working the goods in a boiling bath containing 15 logwood and fustic extracts, working them in a boiling bath containing hematine extract and soap, treating them with hot tannic acid and tartar emetic, and cleansing them in a hot soap solution.
- 20 9. The process of producing washable black silk piece goods which comprises working the goods in a boiling bath containing fustic extract and a logwood extract, adding black iron, blue stone, and acetic acid, working them in a boiling bath containing a logwood extract and soap, treating them with tannic acid and tartar emetic, and cleansing in a hot soap solution.
10. The process of producing washable 25 black silk piece goods which comprises dyeing the goods in a bath containing fustic extract and a logwood extract, working the goods at a boiling temperature, adding black iron, blue stone, and acetic acid to the liquor, working the goods at a boiling temperature, washing, working them in a boiling bath containing a logwood extract and soap, washing, treating them with tannic acid and tartar emetic, cleansing in a boiling soap 30 solution, and then washing and acidulating.
11. The process of producing washable black silk piece goods which comprises dyeing the goods in a bath composed of five hundred gallons water, 30% by weight of fustic extract and 10% by weight of a logwood extract, working the goods in the liquor at a boiling temperature for twenty minutes, adding to the same liquor 25% by weight of black iron, 4% by weight of blue stone, and 20% by weight acetic acid, working the goods at a boiling temperature for one hour, 35 washing, treating in another bath composed of five hundred gallons boiling water, 30% logwood extract, and fifty pounds soap, working them therein for one hour, washing, treating the goods in a bath of five hundred gallons water at 160° F. containing tannic acid in the proportion of six pounds tannic acid per two hundred fifty gallons of dye liquor, treating with tartar 40 emetic in the proportion of four and one-half pounds per two hundred fifty gallons of dye liquor, cleansing in two soap baths at a boiling temperature, and then washing and acidulating.
12. Black silk piece goods dyed in the piece and having the characteristics of fastness to washing in luke warm soap water, evenness in shade, and of not bleeding in cold water or discoloring non-silk fibres.
13. Black silk piece goods dyed in the piece and having the characteristics of fastness to washing in luke warm soap water, evenness in shade, and of not bleeding in cold water or discoloring non-silk fibres, and 45 having antimony in its fibres.

In testimony that I claim the foregoing, I have hereunto set my hand this 21st day of February, 1923.

JOSEPH SEYER.